

## UNITED STATES PATENT OFFICE

2,101,511

SOLE LEATHER AND PROCESS OF PREPAR-  
ING THE SAME

Otto Röhm, Darmstadt, Germany

No Drawing. Application June 29, 1936, Serial  
No. 88,057. In Germany July 2, 1935

6 Claims. (Cl. 149—4)

The invention relates to improvements in sole leather and the process of preparing the same.

Most sole leathers are nowadays prepared with the aid of vegetable tanning agents. The special properties of bark-tanned sole leather are: limited permeability to air, limited water absorption capacity, rapid giving off of water under pressure, limited content of water-soluble substances, and a definite specific gravity. Furthermore, bark-tanned leather increases in strength when it is rolled under heavy pressure, whereas mineral tanned leather becomes softer under such treatment. These properties are of importance in working up the leather for shoe soles and during the wearing of the shoes. During the working up of the leather the important points are that the leather can be sewed and nailed, that the nails hold, and that the cut portions can be finished with a nice gloss. Bark-tanned leather produces, as the worker in the art says: "a good finished trim." When being worn, the properties are manifested by the fact that the wearer does not skid on bark-tanned soles in wet weather, and that the soles, when they become wet, do not swell and thus alter the shape of the shoes.

In order first to shorten the duration of the tanning process and, secondly, in order to be independent of the importation of foreign vegetable tanning agents, the workers in the art have for many years attempted to substitute mineral tanning agents for vegetable tanning agents in the preparation of sole leather, but without appreciable success.

The reason for the lack of success is that the vegetable tanning agents impart the above recited special properties to the leather and these results cannot be achieved with the mineral tanning agents. Even sulphite cellulose extracts have been tried and have been mixed with mineral tanning agents but without result.

It has been found that a sole leather can be obtained in a few days by using a combination employing sulphite cellulose extract, acidified silicic acid solution and a small amount of fatty substances and that such leather possesses all of the properties of bark-tanned leather. The chemicals required in producing this leather need not be imported from abroad.

The method is as follows:

The hides, cleaned as usual, are fulled with sulphite cellulose extract, then treated with an acidified alkali silicate solution and impregnated with a little hard grease such as tallow, paraffin, carnauba wax, synthetic waxes, etc., with or without the addition of solvents.

In order also to make the exterior of the new type of leather simulate bark-tanned leather as much as possible, bichromate may be added to the sulphite cellulose extract, thus producing a leather having a brown color. In lieu of bichromate, other oxidation agents may be used.

## Example

Hides which have been limed, bated, and pickled in the usual manner are fulled in a barrel for two days of eight hours each with:

|                                                                                  | Percent |
|----------------------------------------------------------------------------------|---------|
| Sulphite cellulose extract of 28-30° Bé. (calculated on the weight of the hides) | 50      |
| Sodium or potassium bichromate                                                   | 1 15    |
| Water                                                                            | 25      |

After this period the leathers remain lying on the block for two days. Thereupon they are fulled for two days of eight hours each with:

|                                         | Percent |
|-----------------------------------------|---------|
| Sulphite cellulose extract of 28-30° Bé | 50      |
| Sodium or potassium bichromate          | 1       |
| Water                                   | 25      |

After storing for two days the leathers are fulled for four hours with a solution of:

|                                                 | Percent |
|-------------------------------------------------|---------|
| Formic acid (85%)                               | 4       |
| Waterglass solution having 25% SiO <sub>2</sub> | 10      |
| Water                                           | 15 30   |

until all of the liquor is taken up. The leathers are stored overnight on the block.

Next morning a mixture of 5% paraffin plus 2.5% tetralin is fulled into the leather while in the greasing vat. The leathers, which have been stored on the floor over night are laid out the next morning and dried. Working up proceeds in the same way as in the case of bark-tanned sole leather.

According to the above recited process oxidizing agents such as bichromate are described as used together with the sulphite cellulose extract, and the process so arranged that the leathers are fulled with acid silicic acid solution.

It has also been found that a greatly improved sole leather is obtained if the silicic acid is not used subsequently but rather, under certain conditions, along with the sulphite cellulose tanning process and in such fashion that the hides are first treated with a sulphite cellulose extract liquor without addition of silicic acid and then first with sulphite cellulose liquor containing added silicic acid. Immediately thereupon the leathers are filled with silicic acid solution as de-

40

45

50

55

scribed in the first portion of the present specification.

5 The leathers so prepared may be impregnated with hard greases or waxes or, prior to drying, they may merely be oiled with neat's-foot oil.

The process may with advantage be supplemented by adding small amounts of other tanning agents, such as alum tanning agents, chrome tanning agents, vegetable tanning agents, or synthetic tanning agents, in order to vary the basic character of the leather.

*Examples*

1. Hides which have been limed, bated, and 15 pickled as usual are fulled in a barrel for two days of eight hours each in:

|                                                                     | Percent |
|---------------------------------------------------------------------|---------|
| Sulphite cellulose extract of 28-30 Bé. (calculated on hide weight) | 50      |
| 20 Water                                                            | 25      |

25 After this time the leathers remain lying on the block for two days. Thereupon they are again fulled for two days of eight hours each in a fresh liquor of

|                                                 | Percent |
|-------------------------------------------------|---------|
| Sulphite cellulose extract (of 28-30° Bé.)      | 50      |
| Concentrated formic acid (85%)                  | 2       |
| Waterglass solution having 25% SiO <sub>2</sub> | 10      |
| 30 Water                                        | 25      |

35 After storing for two days the leathers are fulled for 1 to 2 hours with a solution of:

|                                                    | Percent |
|----------------------------------------------------|---------|
| Concentrated formic acid (85%)                     | 4       |
| 35 Waterglass solution having 25% SiO <sub>2</sub> | 10      |
| Mineral oil                                        | 1       |
| Water                                              | 15      |

40 until all of the liquor is taken up. The leathers are stored over night on the block. This fulling 45 may be repeated 1 or 2 times. After the last fulling the leathers are again stored over night on the block and the next morning washed off on both sides with water, laid out, and oiled with neat's-foot oil on the grain side.

45 2. The procedure is that as given in Example 1, with the feature that in preparing the 1st and 2nd tanning liquors 1.5% of chrome alum is added. A sole leather of pleasant color shade is obtained.

50 3. The procedure is that as given in Example 1, with the feature that in preparing the 1st and 2nd tanning liquors, 5% potash alum is added.

A rapid, thorough tanning results and the leather produced has good quality and good tearing strength.

4. The procedure is that as given in Example 1, with the feature that in preparing the 1st and 5 2nd tanning liquors, 10% aluminum formate is added. An especially water-resistant leather is obtained.

5. The procedure is that as given in Example 1, with the feature that in preparing the 1st and 10 2nd tanning liquors, 1% of commercial synthetic tanning agent is added, such as a condensation product of naphthalene sulphonic acid and formaldehyde.

15 The invention has been described in detail for the purpose of illustration but it will be apparent that modifications or variations of the process may be resorted to without departing from the spirit of the invention claimed.

I claim:

20 1. A process for preparing sole leather which comprises first tanning hides with sulphite cellulose extract before any silicic acid is added, and in a subsequent step filling with silicic acid solution.

2. A process for preparing sole leather which comprises first tanning hides with sulphite cellulose extract before any silicic acid is added, and in a subsequent step filling with silicic acid solution, and treating with a member of a group 30 consisting of oils, greases, and waxes.

3. A process for preparing sole leather which comprises first tanning hides with sulphite cellulose extract and an oxidizing agent before any silicic acid is added and in a subsequent step 37 filling with silicic acid solution.

4. A process as set forth in claim 3, wherein the oxidizing agent is a member of a group consisting of sodium bichromate and potassium bichromate.

5. A process for preparing sole leather which 40 comprises first tanning hides with sulphite cellulose extract before any silicic acid is added, then treating with sulphite cellulose extract and silicic acid solution.

6. A process for preparing sole leather which 45 comprises first tanning hides with sulphite cellulose extract before any silicic acid is added, then treating with sulphite cellulose extract and silicic acid solution, and in a subsequent step 50 filling with silicic acid solution.

OTTO RÖHM.